

## UNITED STATES PATENT OFFICE

2,277,544

PROCESS OF PRODUCING FAST DYEINGS  
AND THE DYED FIBER OBTAINED THEREBYErich Fischer and Walter Gmelin, Bad Soden in  
Taunus, and Werner Klst, Konigstein in  
Taunus, Germany, assignors to General Aniline  
& Film Corporation, New York, N. Y., a corpora-  
tion of DelawareNo Drawing. Application November 27, 1940, Se-  
rial No. 367,379. In Germany July 24, 1939

## 8 Claims. (Cl. 8—42)

The present invention relates to a process of producing fast dyeings on cellulose fibers or mixtures of cellulose fibers with animal fibers, and to the dyed fiber obtained thereby.

We have found that dyeings of very good properties of fastness may be obtained on cellulose fibers or mixtures of cellulose fibers with animal fibers, for instance staple fiber from viscose or cuprammonium cellulose and wool, by applying to the fiber a water-soluble pyrazolone-azo-dyestuff which contains in the molecule at least one amino-group capable of being diazotized and at least one grouping capable of forming a metal complex compound, but no hydroxyl group rendering coupling possible, then diazotizing, developing the dyestuff by means of an alkaline treatment and subjecting the dyeings thus obtained to a treatment with an agent yielding metal.

The following examples serve to illustrate the



invention, but they are not intended to limit it thereto:

(1) 1 kilo of a mixed fabric made from 50 parts of wool and 50 parts of staple fiber from viscose is dyed for one hour at 95° C. in a bath containing 40 grams of the azo-dyestuff obtainable by coupling diazotized 1-(4'-amino-benzylamino)-4-hydroxybenzene-3-carboxylic acid with 1-(3'-aminophenyl)-5-pyrazolone-3-carboxylic acid,

40 grams of ammonium sulfate, and  
600 grams of sodium sulfate in

30 liters of water.

The temperature is allowed to fall to 80° C. within 30 to 45 minutes, whereupon the material is rinsed and treated for half an hour in the cold with a solution containing

25 grams of sodium nitrite,  
10 grams of sodium dibutylaphthalenesulfonate and

75 cc. of hydrochloric acid of 20° Bé. in  
30 liters of cold water.

The dyestuff is then developed for half an hour in a bath containing

75 cc. of ammonia of 25 per cent strength and 5 grams of the product obtained by condensation of 1 mol of octodecyl alcohol with 20 mols of ethylene oxide in

30 liters of cold water. The material is then after-treated for one hour at 90° C. with a solution containing

20 grams of chromic fluoride,  
10 grams of glacial acetic acid and  
5 grams of the product obtained by condensation of 1 mol of octodecyl alcohol with 20 mols of ethylene oxide in  
30 liters of water.

15 rinsed and dried. A golden-yellow dyeing of good properties of fastness is obtained.

(2) 1 kilo of a mixture from 50 parts of wool and 50 parts of staple fiber from viscose is treated for one hour at 95° C. in a solution containing

20 40 grams of the azo-dyestuff of the following constitution:



35 (obtainable by coupling 1 mol of 4,4'-bis-[5-oxo-3-methyl - 4<sup>2</sup> - pyrazolyl] - (1) 1-stilbene-2,2'-disulfonic acid which may be obtained from 4,4'-dihydrazino-stilbene-2,2'-disulfonic acid and acetoacetic ester, with 1 mol of diazotized 1-aminobenzene-2-carboxylic acid and 1 mol of diazotized 1-amino-4-nitrobenzene and reducing the nitro-group to the amino-group),

40 10 grams of the product obtained by condensation of 1 mol of octodecyl alcohol with 20 mols of ethylene oxide and

30 80 grams of ammonium sulfate in  
30 liters of water.

45 600 grams of sodium sulfate are then added and the material is allowed to stand for 45 minutes at a temperature falling to 70° C. rinsed and further treated in the manner indicated in Example 1. A yellow dyeing of good properties of fastness is obtained.

(3) 1 kilo of a mixture of 50 parts of wool and 50 parts of staple fiber from viscose is dyed for 55 45 minutes at 90° C. in a bath containing

50 grams of the azo-dyestuff having the following constitution:



(obtainable by coupling diazotized 1-[4'-nitrobenzoylamino]-4-aminobenzene-3-sulfonic acid with 1-[2'-hydroxy-3'-carboxy-5'-sulfophenyl]-3-methyl-5-pyrazolone, reducing the nitro-group to the amino-group, further diazotizing the amino-monoazo-dyestuff obtained and coupling it with 1-[3'-aminophenyl]-3-methyl-5-pyrazolone),

10 grams of the product obtained by condensation of 1 mol of octodecyl alcohol with 20 mols of ethylene oxide,  
40 grams of ammonium sulfate and  
600 grams of sodium sulfate in  
30 liters of water.

The material is allowed to stand for 45 minutes at a temperature falling to 70° C., rinsed, diazotized, developed and after-chromed in the manner indicated in Example 1.

A yellow dyeing of good properties of fastness is obtained.

(4) 1 kilo of a mixture of 50 parts of wool and 50 parts of staple fiber from viscose is dyed for 45 minutes at 90° C. in a bath containing:

30 grams of the azo-dyestuff described in Example 3,  
30 grams of the azo-dyestuff: 1-amino-5-hydroxy-naphthalene-7-sulfonic acid → 1-amino-naphthalene-7-sulfonic acid → 1-amino-naphthalene-7-sulfonic acid,

10 grams of the product obtained by condensation of 1 mol of octodecyl alcohol with 20 mols of ethylene oxide,  
40 grams of ammonium sulfate and  
600 grams of sodium sulfate in  
30 liters of water.



The material is then allowed to stand for 45 minutes at a temperature falling to 70° C., rinsed and further treated for half an hour in the cold with

15 25 grams of sodium nitrite,  
10 grams of sodium dibutylnaphthalenesulfonate and  
75 cc. of hydrochloric acid of 20° Bé. in

20 30 liters of water,

and the dyestuff is developed for half an hour in a bath containing

25 75 cc. of ammonia of 25 per cent strength and  
5 grams of the product obtained by condensation of 1 mol of octodecyl alcohol with 20 mols of ethylene oxide in  
30 liters of cold water.

The material is then after-treated for one hour at 90° C. with a solution containing

30 20 grams of chromic fluoride,  
10 grams of glacial acetic acid and  
5 grams of the product obtained by condensation of 1 mol of octodecyl alcohol with 20 mols of ethylene oxide in  
30 liters of water,

35 rinsed and dried.

A brown dyeing of good properties of fastness is obtained.

The following table indicates the shades of a number of other dyeings obtainable by this invention:

| Parent component                                                                                    | Shade of the dyeing treated with metal salts on mixtures of wool and artificial silk staple fiber |
|-----------------------------------------------------------------------------------------------------|---------------------------------------------------------------------------------------------------|
| <br>1. HO-C6H4-N=N-C(=O)-C(CH3)=N-C(=O)-N1C=CC=C1-SO3H                                              | Treated with chromic fluoride or potassium bichromate: brown.                                     |
| <br>2. HO-C6H4-N=N-C(=O)-C(CH3)=N-C(=O)-N1C=CC=C1-C6H4-C6H4-N=N-C(=O)-C(CH3)=N-C(=O)-N2C=CC=C2-SO3H | Treated with chromic fluoride or potassium bichromate: yellow.                                    |

| Parent component                                                                                                                                                                                                                                                                                                                                                                                            | Shade of the dyeing treated with metal salts on mixtures of wool and artificial silk staple fiber |
|-------------------------------------------------------------------------------------------------------------------------------------------------------------------------------------------------------------------------------------------------------------------------------------------------------------------------------------------------------------------------------------------------------------|---------------------------------------------------------------------------------------------------|
|                                                                                                                                                                                                                                                                                                                                                                                                             | Treated with chromic fluoride or potassium bichromate: brown-orange.                              |
| (obtainable by coupling 1 mol of the bis-pyrazolone from 4,4'-bis-hydrazino-1,1'-diphenyl-2,2'-disulfonic acid and acetoacetic ester, with 1 mol of diazotized 1-amino-4-nitrobenzene-2-carboxylic acid and 1 mol of diazotized 4-amino-4'-hydroxy-1,1'-azobenzene-3'-carboxylic acid and reducing the nitro-group to the amino-group).                                                                     | Treated with chromic fluoride: orange.                                                            |
| 4. 4-amino-1,1'-azobenzene-3-carboxylic acid-4'-sulfonic acid $\longrightarrow$ 1-(3'-aminophenyl)-5-pyrazolone-3-carboxylic acid.                                                                                                                                                                                                                                                                          |                                                                                                   |
| (obtainable by coupling 1 mol of the pyrazolone from the hydrazine of dehydrothiobenzenesulfonic acid and acetoacetic ester, with 1 mol of diazotized 1-amino-2-hydroxy-4-nitrobenzene and reducing the nitro-group to the amino-group).                                                                                                                                                                    | Treated with chromic fluoride: yellowish-brown.                                                   |
| 6. 4-amino-4'-hydroxy-1,1'-azobenzene-3'-carboxylic acid $\longrightarrow$ 1-(3'-amino-phenyl)-5-pyrazolone-3-carboxylic acid.                                                                                                                                                                                                                                                                              | Treated with chromic fluoride: red.                                                               |
|                                                                                                                                                                                                                                                                                                                                                                                                             |                                                                                                   |
| (obtainable by coupling 1 mol of 4,4'-bis-[5-oxo-3-methyl- $\Delta^2$ -pyrazolinyl-(1)]-stilbene-2,2'-disulfonic acid (see Example 2) with 1 mol of diazotized 1-amino-4-hydroxybenzene-3-carboxylic acid and 1 mol of diazotized 1-amino-4-nitrobenzene-2-carboxylic acid and reducing the nitro-group to the amino-group).                                                                                | Treated with potassium bichromate: orange, with chromic fluoride: yellow.                         |
| 8. 1-(4'-aminophenyl)-3-methyl-5-pyrazolone $\longleftarrow$ 2-amino-5-hydroxy-naphthalene-7-sulfonic acid $\longleftarrow$ 1-amino-4-hydroxybenzene-3-carboxylic acid.                                                                                                                                                                                                                                     | Treated with chromic fluoride: brown.                                                             |
|                                                                                                                                                                                                                                                                                                                                                                                                             |                                                                                                   |
| (obtainable by coupling 2 mols of diazotized 5-nitro-2-amino-1-hydroxybenzene-4-sulfonic acid with 1 mol of the urea from 1-(4-aminophenyl)-3-methyl-5-pyrazolone and subsequently reducing the nitro-groups, or by coupling 1 mol of diazotized 5-nitro-2-amino-1-hydroxybenzene-4-sulfonic acid with 1 mol of 1-(4-aminophenyl)-3-methyl-5-pyrazolone, phosgenating and reducing the urea thus obtained). | Treated with copper sulfate: brownish red.                                                        |
| 10.                                                                                                                                                                                                                                                                                                                                                                                                         |                                                                                                   |
| (obtainable by coupling the tetrazo-compound from 1 mol of para-amino-benzoyl-para-phenylenediamine, in an acid medium, with 1 mol of 1-(3'-amino-4'-sulfonyphenyl)-5-pyrazolone-3-carboxylic acid and subsequently coupling the compound obtained with 1 mol of 2-(4'-hydroxy-3'-carboxy-phenyl-sulfonyl)-amino-5-hydroxy-naphthalene-7-sulfonic acid in the presence of sodium carbonate).                | Treated with chromic fluoride: red.                                                               |

**We claim:**

1. A process of producing fast dyeings on fibrous material of the group consisting of cellulose fibers and mixtures of cellulose fibers with

animal fibers, which comprises applying to the fiber a water-soluble pyrazolone-azo-dyestuff selected from the group consisting of mono- and disazo-dyestuffs which contains in the molecule

at least one amino-group capable of being diazotized and at least one grouping capable of forming a metal complex compound, but no hydroxyl group rendering coupling possible, then diazotizing, developing the dyestuff by means of an alkaline treatment and subjecting the dyeings thus obtained to a treatment with an agent yielding metal.



2. A process of producing fast yellow dyeings on fibrous material of the group consisting of cellulose fibers and mixtures of cellulose fibers with animal fibers which comprises applying to the fiber a water-soluble pyrazolone-azo-dyestuff of the following constitution:



then diazotizing, developing the dyestuff by means of an alkaline treatment and subjecting the dyeings thus obtained to a treatment with an agent yielding chromium.

3. A process of producing fast golden-yellow dyeings on fibrous material of the group consisting of cellulose fibers and mixtures of cellulose fibers with animal fibers, which comprises applying to the fiber a water-soluble pyrazolone-azo-dyestuff of the following constitution:



then diazotizing, developing the dyestuff by means of an alkaline treatment and subjecting

the dyeings thus obtained to a treatment with an agent yielding chromium.

4. A process of producing fast brownish-red dyeings on fibrous material of the group consisting of cellulose fibers and mixtures of cellulose fibers with animal fibers which comprises applying to the fiber a water-soluble pyrazolone-azo-dyestuff of the following constitution:



then diazotizing, developing the dyestuff by means of an alkaline treatment and subjecting the dyeings thus obtained to a treatment with an agent yielding copper.

5. Fibrous material of the group consisting of cellulose fibers and mixtures of cellulose fibers



with animal fibers, dyed with a water-soluble pyrazolone-azo-dyestuff selected from the group consisting of mono- and disazo-dyestuffs by the process claimed in claim 1.

6. Fibrous material of the group consisting of cellulose fibers and mixtures of cellulose fibers with animal fibers, dyed with a water-soluble pyrazolone-azo-dyestuff by the process claimed in claim 2.

7. Fibrous material of the group consisting of cellulose fibers and mixtures of cellulose fibers with animal fibers, dyed with a water-soluble pyrazolone-azo-dyestuff by the process claimed in claim 3.

8. Fibrous material of the group consisting of cellulose fibers and mixtures of cellulose fibers with animal fibers, dyed with a water-soluble pyrazolone-azo-dyestuff by the process claimed in claim 4.

ERICH FISCHER.  
WALTER GMELIN.  
WERNER KIRST.